

June 6, 1961

E. BECKER

2,986,876

METHOD OF BURNING BORON CONTAINING FUELS IN A JET  
ENGINE TO MINIMIZE BORON OXIDE DEPOSITS

Filed July 13, 1959



FIG. 1



FIG. 2



FIG. 3



FIG. 4

FIG. 5



FIG. 6

INVENTOR.

EUGENE BECKER

BY

Adams, Forward and McLean

ATTORNEY

1

2,986,876

**METHOD OF BURNING BORON CONTAINING FUELS IN A JET ENGINE TO MINIMIZE BORON OXIDE DEPOSITS**

Engene Becker, Grand Island, N.Y., assignor to Olin Mathieson Chemical Corporation, a corporation of Virginia

Filed July 13, 1959, Ser. No. 826,879  
3 Claims. (Cl. 60—35.4)

This invention relates to a method of minimizing boron oxide deposits on surfaces within jet-type aircraft engines operating on a boron containing fuel. By boron containing fuel is meant a high-energy fuel such as a boron hydride, including diborane, the pentaboranes, and decaborane, organoboranes, including the lower alkyl pentaboranes and lower alkyl decaboranes, and conventional hydrocarbon jet fuels containing the same. Lower alkyl pentaboranes can be prepared, for example, according to the method described in application Serial No. 546,803, filed November 14, 1955, now abandoned, of Jack R. Gould and John E. Paustian. Lower alkyl decaboranes can be prepared, for example, according to the method described in application Serial No. 557,634, filed January 6, 1956 to Joseph A. Neff and Edward J. Wandel.

The present invention can be applied to any of the three basic types of jet engines, i.e. the ram-jet, the turbo-jet, and the turbo-prop, although it has a particular application to the turbo-jet and turbo-prop type engines, and will be further described as applied to a turbo-jet engine.

In the operation of a turbo-jet aircraft engine, air flows into the engine through the air entrance section and then into the compressor section, where it is usually compressed to a pressure of about 45 to 180 p.s.i.g. The air entrance and compressor section may follow any one of several designs; and the compressor section may possess either an axial or a centrifugal compressor. If of the centrifugal type, the compressor may additionally possess either a single or a double entry.

From the compressor section, the compressed air flows into the combustion section where it is combined with a metered and atomized or prevaporized amount of fuel and its temperature increased by combustion of the fuel. It will be noted that the air flow in this section is such that only a relatively small amount of the air actually mixes with the fuel at the point of combustion. This portion of the air is generally referred to as the primary air supply. The weight ratio of primary air to fuel is generally between 10 to 1 and 50 to 1.

Following the combustion of the fuel, the combustion products are almost immediately and intimately mixed with the remaining or secondary air. Thus, the combustion products are cooled from a combustion temperature of about 3500° to 4000° F. to an average temperature of about 1400° F. The latter temperature is dictated at the present time by the types of metals and metal alloys that are presently available for use within the turbine section of an engine.

The gaseous products of combustion and the excess air entering the turbine section from the combustion section cause the turbine rotor or rotors to revolve and to drive the compressor in the compression section and also auxiliary equipment such as fuel pumps, lube oil pumps, generators, etc.

The gases leaving the turbine then flow into the tailpipe section from whence they vent to the atmosphere. The design of this section may vary considerably. For example, it may have either a single or double exit, and it may also be of the variable orifice or adjustable exhaust nozzle type. When the tailpipe is provided with an afterburner, it is essential that a variable exhaust

2

opening be provided to adjust for both normal and after-burning combustion conditions. The tailpipe section normally operates at temperatures of about 900° to 1400° F.

When afterburner nozzles are provided in the tailpipe section, a diffuser is usually placed between the turbine section and the nozzles. This device serves to redistribute the gas flow in the tailpipe and to promote better combustion of the fuel issuing from the afterburner nozzles.

10 The combustion section may be any one of the conventional types as, for example, one that employs multiple combustion chambers ("cans") or one that uses an annular combustion liner or chamber (a "burner basket"). In the first of these types, the air flow is split upon leaving the compressor and equal portions sent to each can, where these portions are combusted with portions of the fuel. The combustion products are then recombined with secondary air and routed to the turbine section.

When the combustion section is of the burner basket type, the primary portion of the air is diverted from the main stream and directed toward the fuel injector within the basket where it burns with the fuel. The remaining or secondary air is then mixed with the products of combustion at a point prior to their entrance into the turbine section.

25 The turbine section of a jet engine may contain one or more turbine rotors and one or more stages. In addition, the turbine blades may be of the impulse and/or reaction types and may or may not be shrouded. Associated with the turbine rotor blades are stator blades which direct the hot gases against the rotor blades.

30 One of the more serious problems associated with the use of boron containing fuels in turbo-jet aircraft engines results from the formation of boron oxide as a combustion product and its subsequent deposition on the surfaces of the combustion section, the turbine section, and the tailpipe section. For example, a pound of diborane produces 2.5 pounds of  $B_2O_3$  and a pound of pentaborane, 2.76 pounds. The glass-like boron oxide 35 has an approximate melting point of 840° F. and has a high viscosity at turbine operating temperatures of about 1400° to 1600° F. Thus boron oxide deposits collect and flow along engine parts, including combustor walls and transition pieces, turbine rotor and stator blades, tailpipe walls, including afterburner parts, and variable-area nozzles.

40 It has been proposed to minimize deposits of boron oxide in turbo-jet engines by avoiding the strong reverse flow that is usually designed into a high velocity combustor to provide flame piloting. The wide flammability 45 limits and high flame speeds of boron fuels make it possible to reduce the piloting otherwise required by hydrocarbon fuels. It has also been proposed to minimize boron oxide deposits by filming the combustor walls with air to prevent impingement of boron oxide on the surfaces thereof. Various methods of providing the air film are available such as porous walls, louvers, step construction, etc. These proposals, however, have not been successful in alleviating the boron oxide deposition problem.

50 In accordance with the present invention, boron oxide 55 deposits are minimized within the combustion, turbine and exhaust sections of an air-breathing jet-type aircraft engine operating on a boron containing fuel by introducing a normally liquid ether of silicon wherein the ratio of silicon to oxygen is within the range of 0.5 to 4 within the appropriate section.

The silicon ether can be introduced within those sections where boron oxide is prone to form by any one or more of several known means including introduction 65 within the air or combustion gas stream flowing to the pertinent sections and introduction directly into the per-

tinent sections. The silicon ether can be introduced within the combustion section, for example, by incorporation into the primary or secondary air stream from the compressor section. The silicon ether can be introduced within the turbine section, for example, by direct injection as by utilizing a porous material, such as a ceramic material or sintered stainless steel, for construction of the turbine stator blades and transpiring the silicon ether through the stator blades. The silicon ether can be introduced within the exhaust section by direct injection into the gas stream flowing therein. Where an afterburner is employed, the silicon ether can be injected at or subsequent to the diffuser and also in the air stream supplied to the afterburner.

In order to test the efficiency of silicon ethers in minimizing the deposit of boric oxide on heated surfaces, a combustion and exhaust system simulating that of a jet-type engine was constructed and is shown in the attached drawing wherein FIGURE 1 is a side elevation and FIGURE 2 is an isometric of the combustion and exhaust system, FIGURE 3 is a section along line A—A of FIGURE 1, FIGURE 4 is a section along line B—B of FIGURE 1, FIGURE 6 is a section along line C—C of FIGURE 1 and FIGURE 5 is a section along line D—D of FIGURE 4.

In the drawing numeral 1 represents a section of four inch diameter stainless steel pipe about sixty-eight inches long and divided into four sections by flanges 2, 3, 4 and 5. Attached to pipe 1 by means of flange 6 was an eight inch diameter section of stainless steel pipe about 10 inches long defining the exhaust chamber.

The section of pipe 1 between flanges 2 and 3 had disposed therein an Inconel liner 8, defining the combustor, with an average diameter of 3.12 inches which tapered outwardly toward flange 3 one-eighth inch per foot and was two feet long. Liner 8 was perforated and contained eighty holes varying from three-sixteenths inch to three-eighths inch in diameter. Air entered the combustor through inlets 9 and 9a. The bulk of the air entered inlet 9 at 160° F. JP-4 fuel was injected into the combustor by means of inlet 10 and boron containing fuel was injected into the combustor by means of inlet 11. Inlet 11 was connected to a standard 80° hollow cone oil burner nozzle and inlets 9a and 10 were connected to a fuel-air nozzle which injected the mixture into the combustor by means of an annular opening around the burner nozzle. The fuel-air mixture was ignited by means of a high energy, high voltage, air-gap type spark plug 12.

The section of pipe 1 between flanges 3 and 4 was fourteen inches long. Two inches upstream from flange 4 was thermocouple bank 13 consisting of two thermocouples.

The section of pipe 1 between flanges 4 and 5 was ten inches and defined the test section which contained three Vycor-glass windows and a probe port located circumferentially around pipe 1 midway in the test section. Through the probe port was inserted deposition probe 14 which consisted of a section of one-half inch stainless steel tubing with the base closed by welding. The leading edge had a projected deposition area of 1.5 square inches. Probe 14 was attached to pipe 1 by a stainless steel flare. Just upstream of and parallel to probe 14 was silicon ether inlet 15 communicating with reservoir 16. Nitrogen pressure, usually 0.5 to 1.0 p.s.i., was applied to reservoir 16 by means of line 17. The flow rate of the silicon ether was controlled by varying the nitrogen pressure applied to the reservoir.

The section of pipe 1 between flanges 5 and 6 was ten inches long. Six and one-half inches downstream from flange 5 was thermocouple bank 18 consisting of eight thermocouples.

This combustion and exhaust system was employed in each of the following examples.

#### Example I

Air flow through inlets 9 and 9a is established and JP-4 is injected through inlet 10 and burned in the combustor at the flow rate required to provide an exhaust gas temperature of 1500° F. measured by thermocouple bank 18. Operation with JP-4 alone is continued for a preheating period of five minutes. A mixture of trimethoxyboroxine and acetone (4 parts trimethoxyboroxine and 1 part acetone) is then injected into the combustor through inlet 11 at a flow rate of 0.0055 pound per second for intervals of three, four or five minutes, the JP-4 flow rate being adjusted to maintain a temperature of 1500° F. at thermocouple bank 18. At the end of the three, four and five minute intervals of trimethoxyboroxine flow, JP-4 combustion is continued for thirty seconds at which time the deposition probe 14 is removed and weighed. By this means it is determined that the boric oxide deposition rate on the probe is 0.06 pound per hour.

The probe is cleaned and replaced and the system again brought to preheat temperature with JP-4. A Dow-Corning dimethyl silicone fluid having a viscosity at 25° C. of 90 centistokes is then charged to reservoir 16 and nitrogen pressure is applied until a flow of silicone fluid through inlet 15 is established sufficient to wet the leading edge of the probe as observed through the Vycor glass windows. The trimethoxyboroxine-acetone flow is then started, the JP-4 flow rate being adjusted to maintain a temperature of 1500° F. at thermocouple bank 18. The experiment is continued for about 4.5 minutes until all of the silicone fluid has been expended. As observed through the Vycor glass windows, the silicone fluid is effective in preventing boron oxide deposition on the portions of the probe wetted by the silicone fluid.

The test conditions are summarized as follows:

|                         |                 |
|-------------------------|-----------------|
| Trimethoxyboroxine flow | 0.0055 lb./sec. |
| Air flow                | 0.25 lb./sec.   |
| Stream temperature      | 1480° F.        |
| Length of test          | 4.5 minutes.    |
| Silicone fluid flow     | 44 grams/min.   |

#### Example II

This experiment was carried out in a manner similar to Example I except that tetraethoxysilane is employed instead of the silicone fluid. As observed through the Vycor glass windows, the tetraethoxysilane is also effective in preventing boron oxide deposition on the probe.

In place of the tetraethoxysilane employed in Example II, other lower alkoxy silanes can be employed such as tetramethoxysilane, dimethyldiethoxysilane, ethyltriethoxysilane, amyltriethoxysilane, and vinyltriethoxysilane. The hydrolysis and condensation or polymerization products obtained by the controlled hydrolysis of the alkoxy silanes or aryloxy silanes with water can also be employed. Note U.S. Patent 2,416,503 and 2,416,504 to Trautman et al. for a description of these materials.

In place of the silicone fluid employed in Example I, other silicone fluids of lower and higher molecular weight can be employed, such as those described as the "first type" in U.S. Patent 2,765,221 to Lusebrink et al., including hexamethyl disiloxane with a viscosity of 0.65 centistoke at 25° C. to polysiloxanes having a viscosity as high as 60,000 centistokes or more at 25° C. These silicone fluids are generally produced by condensing dialkylsilanediols or diarylsilanediols, or mixtures thereof, wherein the alkyl and aryl groups contain 1 to 7 carbon atoms, and then endblocking the polymer by admixing therewith a trialkyl or triarylsilanol. Also the cross-linked polymers obtained, for example, by condensing a mixture of organo-silane triols with organo-silane diols and organo-silanols or both, as described in above mentioned U.S. Patents 2,416,503; 2,416,504 and 2,765,221 can be employed.

The amount of silicon ether required to be introduced within the various sections of the engine in order to minimize the deposition of boric oxide varies with the characteristics of the engine and the conditions under which it operates. For example, in ram-jets, where a lesser deposit problem exists than in turbo-jets, less silicon ether is required. In general, however, the total amount of silicon ether introduced within the various engine sections is sufficient to maintain the deposition of boric oxide desirably low.

I claim:

1. A method of minimizing boron oxide deposits within the combustion, turbine and exhaust sections of an air-breathing jet-type aircraft engine operating on a fuel containing at least one material selected from the class consisting of boranes and organoboranes which consists

of introducing within such a section in contact with surfaces upon which boron oxide would normally deposit a normally liquid ether of silicon wherein the ratio of silicon to oxygen is within the range of 0.5 to 4 in an amount sufficient to minimize boron oxide deposition.

5 2. The method of claim 1 wherein the silicon ether is tetraethoxysilane.

3. The method of claim 1 wherein the silicon ether is a dimethyl silicone fluid having a viscosity of 90 centi-  
10 strokes at 25° C.

References Cited in the file of this patent

15 Proell et al., The Journal of Space Flight, vol 2, No. 1, Jan. 1950, pages 1-9, at page 2. (Copy in Scientific Library.)